

# UNITED STATES PATENT OFFICE.

FREDERICK E. BLAISDELL, OF CAMDEN, NEW JERSEY, ASSIGNOR TO THE  
SIL-CRUSTA MANUFACTURING COMPANY, OF SAME PLACE.

## INSULATING COMPOSITION.

SPECIFICATION forming part of Letters Patent No. 440,391, dated November 11, 1890.

Application filed May 3, 1890. Serial No. 350,513. (No specimens.)

*To all whom it may concern:*

Be it known that I, FREDERICK E. BLAISDELL, a citizen of the United States, residing at the city of Camden, in the county of Camden and State of New Jersey, have invented 5 a certain new and Improved Insulating Composition, of which the following is a specification.

My invention relates to a new and improved 10 compound or material for insulating devices, especially electrical machines and instruments — for instance, such as the contact pieces of switches for electric circuits—as well as in connection with electric cut-outs for 15 lamps and other electrical appliances.

The principal object of the invention is to provide an inexpensive, durable, and efficient 20 insulating compound, substance, or material which may be readily molded or otherwise formed into any desired shape or configuration for use.

My invention consists of an insulating composition for electrical and other purposes, as hereinafter fully described.

The body or interior portion of the insulating 25 material, substance, or compound is composed of powdered asbestos and plastic clay thoroughly mixed in a dry state or condition and in the following proportions: seventy- 30 two parts of asbestos and eighteen parts of plastic clay, by weight, more or less. The dry mixture of asbestos and clay is then mixed

with a suitable flux—for example, a flux containing six parts of powdered borax and four parts of powdered feldspar, by weight, more 35 or less. Of course instead of using this flux containing borax and feldspar in the proportions above described, other equivalent fluxes may be used; but good results have been obtained in practice by using a flux containing 40 feldspar and borax, and therefore preference is given to these materials.

Among the many advantages possessed by the above-described insulating compound or material the following may be particularly 45 mentioned: low electrical conductivity due to the high percentage of asbestos contained therein and the cheapness or the cost of production thereof.

Having thus described the nature and objects 50 of my invention, what I claim as new, and desire to secure by Letters Patent, is—

An insulating composition for electrical and other purposes, composed of asbestos, 55 clay, and a flux, as feldspar and borax, substantially as and for the purposes described.

In witness whereof I have hereunto set my signature, in the presence of two subscribing witnesses, this 1st day of May, A. D. 1890.

FRED. E. BLAISDELL.

Witnesses:

HERMANN BORMANN,  
THOMAS M. SMITH.